

Patented June 21, 1927.

1,632,829

# UNITED STATES PATENT OFFICE.

HANS FLEISSNER, OF LEOBEN, AUSTRIA.

## METHOD OF DRYING COAL AND THE LIKE.

No Drawing. Application filed January 11, 1926, Serial No. 80,665, and in Austria August 14, 1924.

This invention relates to an improved method of drying coal and the like.

It frequently happens that fuels, particularly in the case of brown-coal containing a large quantity of water, fall to pieces on being dried. This occurrence depends on the colloidal character of the fuel. At first the outermost layers dry up to a great extent and subsequently drop off, whereafter the same procedure is repeated with respect to the next layers until the entire fuel has fallen to pieces. In order to avoid this, it has already been proposed to heat the coal above atmospheric pressure for some time 10 in closed sheet-metal boilers.

Further it has been proposed to gradually heat the materials to be dried at first with a vapor-laden atmosphere but at a temperature below the vaporizing temperature 20 of the moisture, and thereafter accelerating the drying operation, which is very slow at the beginning, by condensing the moisture of the air which is again returned and re-heated during the circulation.

According to the present invention this drawback is avoided in that the colloidal character of the material is abolished as far as possible before the drying operation. This may be accomplished by some sort of 30 coagulation of the colloids, if the coals are heated to a higher temperature and thereby care is taken, that water does not escape from the coal during this procedure. In carrying out the invention, first the coal is heated up to drying temperature in the presence of steam or by the latter, whereby care is to be taken, that the partial pressure of the steam above the fuel to be dried is so great, that the water cannot escape from 35 the coal during the heating. In order to attain this, it is only necessary to pass saturated steam of a suitable temperature over the coal, until the same has taken on the temperature required for the drying. Only after the coal has been subjected in this manner for some time to the necessary drying temperature, the water is allowed to escape from the coal by progressively reducing the steam-pressure, and now the coal is 40 drying quickly. For this object air is now passed over the coal, so that a progressive reduction of the steam-pressure takes place and the coal is dried quite uniformly without falling to pieces.

A suitable apparatus for carrying out the present invention is diagrammatically illus-

trated by way of example in the accompanying drawing.

In the drawing, 1 indicates a closed drying chamber, provided with an inclined perforated bottom 2, the lower end of which leads to a discharge opening 3, which is adapted to be closed. The top end of the drying chamber terminates in a funnel 4, which can be closed. A pipe 5 for supplying saturated steam and a pipe 6 for hot air communicate with the interior of the chamber 1 underneath the perforated bottom 2, and both pipes are furnished with closing members. A pipe 7 for discharging the vapors and gases is connected to the top of the drying chamber.

For carrying out the method, saturated steam is supplied for such a length of time, until the brown coal is heated to about 100° 75 Celsius, without losing the moisture. At this temperature the brown coal loses its colloidal character. The steam and hot air are discharged through the pipe 7 and for the better utilization of heat can be supplied 80 to a battery of drying chambers after suitably separating the moisture and re-heating the same underneath the perforated bottom. After the material is completely dried, the same is discharged through the opening 3.

The temperature, steam pressure and time of action differs according to the moisture-content and place of origin of the coal. For instance brown-coal from the Alexander mine in Bohemia is heated for about three quarters of an hour at a pressure of 3 atmospheres, corresponding to about 130° centigrade and subsequently is dried for about 2 hours by reducing the partial steam pressure. The coal from the Koflacher mine in 95 Austria contains a considerably greater quantity of water and calls for a pressure of about 15 atmospheres corresponding to about 197° centigrade and a steam treatment for about one hour, and subsequently 100 has to be dried between 2 and 3 hours.

I claim:-

1. Method of drying coal and the like consisting in first heating the coal for about one hour in the presence of steam of a pressure ranging from 3 atmospheres corresponding to a temperature of about 130° centigrade to 25 atmospheres corresponding to a temperature of about 235° centigrade thus preventing the escape of water from the coal, thereafter progressively reducing the pressure of the steam in order to start 105 110

the drying, and continuing this reduction until the coal is dry.

2. Method of drying coal and the like consisting in first heating the coal for about one hour by means of steam of a pressure ranging from 3 atmospheres corresponding to a temperature of about 130° centigrade to 25 atmospheres corresponding to a tem-

perature of about 235° centigrade thus preventing the escape of water from the coal, <sup>10</sup> thereafter progressively reducing the pressure of the steam in order to start the drying, and continuing this reduction until the coal is dry.

In testimony whereof I affix my signature.  
DR. HANS FLEISSNER.